

March 26, 1974

J. E. YOUNG

3,799,776

METHOD AND MATERIALS FOR PHOTOGRAPHIC COLOR IMAGING

Filed May 19, 1972



1

3,799,776

## METHOD AND MATERIALS FOR PHOTOGRAPHIC COLOR IMAGING

James E. Young, 50 Larchwood Drive,  
Pittsford, N.Y. 14534

Continuation-in-part of abandoned application Ser. No. 52,820, July 7, 1970. This application May 19, 1972, Ser. No. 254,932.

Int. Cl. G03c 1/40, 1/72, 7/00

U.S. Cl. 96—2

14 Claims

### ABSTRACT OF THE DISCLOSURE

Color imaging methodology and materials are disclosed utilizing cyanine dye coordinate structures of the type:



where  $M$  is a heavy metal ion and  $n$  is an integer, said structure being chosen to be light sensitive to a selected color component of a light pattern to be imaged, where  $Z$  is a dye coupler for the developer-color former fragment  $\Delta NH$  and which when coupled with said fragment yields a dye having a desired color relationship to said selected color component.

This application is a continuation-in-part of my co-pending application, Ser. No. 52,820, filed July 7, 1970 now abandoned.

This invention relates generally to imaging technology, and more specifically relates to methods and materials for color imaging of light patterns.

Virtually all presently employed chemically-based imaging systems, including the trademark-identified systems of Kodacolor (negative), Kodachrome and Ektachrome Reversal (positive), and Polaroid Dye Transfer Reversal color, utilize a so-called "monopack" tri-emulsion system. These monopack systems are structurally very complex and in particular are typically composed of three superimposed thin emulsion layers, sensitive respectively to blue, green, and red light, plus a suitably interposed yellow dye layer and a plastic support substrate. Each emulsion layer therein contains specific color sensitizers — commonly cyanine dyes — specific color couplers (to form direct or complementary colors), silver halide crystals, sensitizers, retarders, etc.

In the newer of these conventional color imaging systems, the said color couplers are introduced into the recording emulsion and prevented from migrating by incorporating the coupler in an oil emulsion or resin and suspending small particles of the emulsion or resin throughout each monopack emulsion layer. The color former-developing agent, usually a substituted para-phenylene diamine, is contained in a separately employed color developer solution. The color former-developing agent therefore must diffuse through the multi-layer emulsion, reduce the exposed silver to in turn oxidize the developing agent, whereupon the oxidized developing agent couples with the emulsion-contained coupler to form the appropriate dyes. In consequence of such arrangement considerable resolution is lost in current color films, and scattering effected by the aforementioned small particles additionally has a detrimental effect on color rendition of the materials.

2

Developing processes for such conventional color imaging systems are furthermore well-known to be very complex and time-consuming. By way of illustration, and even reducing such processes to their simplest form, at least the following sequential steps are involved in development of a conventional positive (reversal) color film: negative silver development; stop washing; white light exposure; dye former development; silver bleach; stop-washing; hypo fixing; and wash and drying.

In accordance with the foregoing, it may be regarded as an object of the present invention, to provide processes and materials which vastly simplify both the structuring of color imaging members and the processing techniques for producing color images in an exposed member.

It is a further object of the present invention, to provide color imaging methods and materials which enable development of color images in exposed members by simple heat, infra-red or radiant energy processing techniques, or by simple treatment of said member with a buffered aqueous alkaline solution.

It is another object of the present invention, to provide a color imaging member wherein a single layer in the member may carry commonly the various color-sensitive compounds of the invention, with in situ formation of the dye image occurring in such layer without the use of a migrating dye former-developing agent, whereby a vast improvement in color image resolution and color rendition is enabled.

Now in accordance with the present invention, the foregoing objects, and others as will become apparent in the course of the ensuing specification, are achieved in a color imaging system based upon the use of cyanine dye coordinate structures of the general type:

(1)



where  $M$  is a heavy metal ion such as silver (which ion may also be thus complexed as the metal halide),  $n$  is an integer, and  $Z$  is a dye coupler for the developer-color former fragment  $\Delta NH$ . In systems in accordance with the invention the said coordinate structure is chosen to be light sensitive to a selected color component of a light pattern to be imaged, with  $Z$  being an appropriate coupler for  $\Delta NH$  such that when coupled therewith a dye results having a desired color relationship to said selected color component. Impingement of light including said selected color component—i.e. conventional exposure—serves to

reduce the metallic ion  $M$  and to oxidize the fragment  $\Delta NH$ . Thereafter development of the desired dye image may be simply brought about by disrupting—e.g. by radiation or chemical environment—the chemical bonds joining the developer fragments to the dye coordinate structure, whereby the dye coupler  $Z$  couples with oxidized developer fragments at points exposed to said selected color component. Because the coordinate structures depicted effectively carry in a single organic salt form the light sensitizer (and light-sensitive) agent, developer-color former, and dye coupler, production of the ultimately desired dye image is entirely in situ, i.e. in the immediate vicinity of the dye structure (1); thus unlike the practice in conventional color photography no external developing agent need in any way be utilized. The result is a vast simplification in developing techniques and in image resolution resulting from development: and moreover a "tri-mix" emulsion is enabled, which is to say

60

65

70

a color imaging member wherein a single layer carries simultaneously and commonly several or a plurality of classes of coordinate structures of the aforementioned type sensitive respectively to different color compounds of an incident light image.

In the drawings appended hereto:

FIG. 1 is a schematic cross-section through a reversal positive monopack color film based upon present invention; and

FIG. 2 depicts in schematic cross-section a color film structure which in accordance with the invention utilizes but a single sensitized layer.

The coordinate structures utilized in accordance with the invention are in an organic structural sense, members of dye sensitizers classified as cyanines, azacyanines, carbocyanines, hemicyanines, and merocyanines, and contain heat or alkaline fracturable members which when released act in the nature of photographic developer-color formers. The fact that these compounds are thus per se dye sensitizers accounts for the fact that no additional agents need be present in imaging members incorporating these coordinate structures to perform the sensitization function.

The said coordinate structures may also, in a structural sense, be regarded as derivatives of the compound guanidine. Considering the structures as such, we may note by way of illustration the action of heat (typically 100 to 200° C.) or alkaline conditions (pH of about 10 to 13) upon a representative triphenyl guanidine:



In this illustration, the symmetrically paired double substituted paraphenylen diamines to the left of the carbon atom correspond to the  $\Delta\text{NH}$  fragment; the group



corresponds to the coupler which is more generally represented by Z in the generalized coordinate structure (1). The broken lines shown as intersecting the C—NH bonds depict where bond fracturing in the illustrated compound occurs in the presence of heat-application or of highly alkaline (pH of 10 to 13) conditions.

If we consider the case where the illustrated compound is complexed with a heavy metal such as silver (which could be derived too from complexing with a silver halide), the double substituted paraphenylen diamine groups are oxidized where previously struck by activating (or "actinic") light wavelengths to yield:



quinone diamine groups. Since quinone groups are in condition to thus couple with the Z-corresponding group to yield a preselected dye if the Z-group is appropriately chosen.

More generally in accordance with the invention, the coordination compound silver salt (or silver halide salt) (1) of the cyanine organic dye acts as the sensitive medium, color sensitizer, dye coupler (direct or complementary color), and developing agent. All of these functions are incorporated in the sensitive layer as one coordination compound. The system can also use other heavy metals, in addition to silver, as electron traps or redox components.

An exemplary structure of these multipurpose cyanine dye coordinate structures is as follows:



The bracket beneath the structure (2) indicates that the entire structure per se is a cyanine dye sensitizer. The left-hand—guanidine-like—portion of the dye coordinate structure may be bonded to the coupler structure Z to provide resonance interaction (conjugated) or in an inert position (unconjugated or blocked) to prevent resonance interaction to provide the desired color in the cyanine sensitizer. In this exemplary structure  $\Delta\text{NH}$  of structure (1) is shown as a double substituted paraphenylen diamine. While such is indeed a preferred form for  $\Delta\text{NH}$  it will be appreciated that in general  $\Delta\text{NH}$  can comprise virtually any of the numerous color former-developing agents known to those skilled in the art of color photography. Thus in more general terms the coordinate structure (2) can be written as:



where

55 R=alkyl, aryl, H,  $\text{CH}_3$ ,  $\text{C}_2\text{H}_5$ ,  $\text{C}_2\text{H}_5\text{CH}_2$ ,  $(\text{CH}_2)_n\text{OH}$ ,  
 $-\text{CH}_2\text{C}_6\text{H}_4\text{SO}_3\text{H}$ ,  $-(\text{CH}_2)_n\text{CO}_2\text{H}$ ,  
 $-(\text{CH}_2)_n\text{NHSO}_2\text{CH}_3$

60  $-(\text{CH}_3)_n\text{OO}_2\text{SOH}$ ,  $-(\text{CH}_2)_n\text{OC}_6\text{H}_4\text{SO}_3\text{H}$ ,  
 $-\text{C}_3\text{H}_6\text{SO}_3\text{H}$

$-\text{CH}_2\text{OCH}_2\text{OH}$ ,

65  $\begin{array}{c} \text{CH}_2 \\ | \\ -\text{N}-\text{O}-\text{CH}_2- \end{array}$  and  $\begin{array}{c} \text{CH}_2\text{CH}_2 \\ | \\ -\text{CH}-\text{O}-\text{CH}_2- \end{array}$

70  $\text{R}'=-\text{NR}_2$ , and  
 $\text{R}''=\text{R}$ ,  $-\text{OR}$ ,  $-\text{NR}_2$



75 It may, among other things, be observed in (3) that the two components corresponding to the  $\Delta\text{NH}$  in structure (1) can differ from one another; thus the two  $\Delta\text{NH}$  frag-

ments in (1) can represent differing developer-color formers.

Furthermore it will be appreciated that the dye coupler Z in structure (3), may itself be chosen with enormous flexibility, so that when coupler Z—which may also be referred to as a “dye intermediate”—couples with the color former-developer ANH, a dye results which has specifically desired color characteristics with respect to the original actinic radiation which activated the coordinate structure.

The dyes used herein are by virtue of their dual purpose modified cyanines. Dyes of this general type are elucidated in the literature and the procedures for synthesis of compounds of this type are well-known to those skilled in the art. Many current processes, for example, for the formulation of cyanine dyes use condensation type reactions. These reactions, shown in “Mees, C. E. K., The Theory of the Photographic Process, The Macmillan Co., New York, 1954,” utilize an active hydrogen on one reactant and an active negative atom (halogen, cyano, alkyl or aryl mercapto, alkoxy, anilino, or acetanilido) on the other reactant. Condensing agents are used as scavengers and to shift the reaction equilibrium in the desired direction. The intermediates used in the preparation of conventional sensitizing dyes, and the condensing agents, including their preparative procedures, are discussed in “Glafkides, P., Photographic Chemistry, vol. I and II, Fountain Press, London, 1960” starting on page 753.

Typically, the dyes described in this patent application can be prepared by the two following exemplary approaches, depending upon the substituents in the dye intermediates:

(a) by condensation of appropriately substituted guanidines with intermediates containing negative active atoms in the desired positions; and (b) by formation of the appropriately substituted guanidine structure in situ via the reaction of the substituted carbodiimide with amino group(s) located in the dye intermediate.

The general scheme pursuant to which synthesis of the dye sensitizers of the invention may be effected, is set forth as follows:

5 may require cooling to contain the reactants. After the initial reaction subsides, attach electric heating mantle and water cooled condenser. Reflux the mixture for 8 hours. Distill off the excess  $\text{CS}_2$  and alcohol. Wash residue with an excess of dilute  $\text{HCl}$  (1:10) to neutralize the residual  $\text{KOH}$  and remove unreacted para phenylene diamine. Filter, wash with warm water, and dry. Purify by recrystallization, desolving the residue under reflux in boiling rectified spirits (Ethanol). Filter in heated funnel if the solution is not clear. Add hot water until the solution becomes cloudy, cool, and filter.

10  $\text{N},\text{N}''$  bis (4-dimethylaminophenyl) thiourea is also available commercially as #2239 from: K&K Laboratories Inc., Plainview, N.Y.

## EXAMPLE 2

### (II) Preparation of $\text{N},\text{N}'$ bis (4-dimethylaminophenyl)carbodiimide

Equations:



25 In a 500 ml. balloon flask mix 100 ml. (87.9 g.) of anhydrous benzene (Baker 9154) (alternate solvents diethyl ether or acetone), 65 g. anhydrous calcium chloride (Baker 1314) (alternate drying agents: Sodium sulphate (Baker 3891), magnesium sulphate (Baker 2506), or anhydrous magnesium carbonate), 59.5 g. of  $\text{N},\text{N}'$  bis (4-dimethylaminophenyl) thiourea (from preparation I or K&K Laboratories #2239), and 144 g. of mercuric oxide (Baker 2620 or 2630) (alternate desulfurization agents: lead oxide (Baker 2338) or sodium hypochlorite). Attach

30 electric heating mantle and water cooled condenser. Reflux the mixture for 6-8 hours. Filter to remove sulphides and drying agent, distill off excess benzene, and dry. Purify by recrystallization from dry benzene. *Maintain the compound in a dry atmosphere to prevent the formation of urea compounds.*

35 40

## SYNTHETIC FLOW CHART



<sup>1</sup> Commercially available chemicals.

Detailed procedures respecting preparation of the said sensitizers pursuant to the foregoing flow chart are set forth hereinbelow:

## EXAMPLE 1

### (I) Preparation of $\text{N},\text{N}'$ -bis(4-dimethylaminophenyl) thiourea

Equations:



In a 500 ml. balloon flask, mix 63.5 ml. (50 g.) absolute ethyl alcohol, 45 ml. (57 g.) Carbon disulfide (Baker 2630), 132 ml. (136 g.)  $\text{N},\text{N}$  dimethyl-p-phenylene diamine (EK P 2147) and 11.4 g. Potassium Hydroxide (Baker 3140). An exothermic reaction takes place which

Bis (p-dimethylaminophenyl) carbodiimide is also commercially available as #12325 from K&K Laboratories Inc., Plainview, N.Y. See also Pat. 2,942,025.

## EXAMPLE 3

### (IIIa) Preparation of $\text{N},\text{N}'$ bis (4-dimethylaminophenyl) guanidine—from carbodiimide

Equations:



In a 500 ml. balloon flask add 25 g. of anhydrous calcium chloride (Baker 1314) (alternate: sodium sulphate (Baker 3891), magnesium carbonate—anhydrous, or mag-

nesium sulphate (Baker 2506), 100 ml. (87.9 g.) dry benzene (Baker 9154), and 93.5 g. of N,N' bis (4-dimethylaminophenyl) carbodiimide (from preparation II or #12325 from K&K Laboratories Inc.). A gas dispersion tube with fritted disc or cylinder is introduced into the mixture and anhydrous ammonia gas is allowed to bubble through the liquid at room temperature for 30 minutes. Filter to remove the drying agent and distill off the benzene exercising care to prevent thermal decomposition of the guanidine. Purify by recrystallization from dry benzene or absolute ethanol.

#### EXAMPLE 4

(IIIb) Preparation of N,N' bis (4-dimethylaminophenyl) guanidine—direct from thiourea

Equations:



In a 500 ml. 2 neck balloon flask mix 100 ml. (87.9 g.) of anhydrous benzene (Baker 9154) (alternate solvents: diethyl ether or acetone), 65 g. anhydrous calcium chloride (Baker 1314) (alternate drying agents: sodium sulphate, Baker 3891, magnesium sulphate, Baker 2506, or anhydrous magnesium carbonate), 59.5 g. of N,N' bis (4-dimethylaminophenyl) thiourea (from preparation I or K&K Laboratories #2239) and 144 g. of mercuric oxide (Baker 2620 or 2630) (alternate desulfurization agents: lead oxide, Baker 2338, or sodium hypochlorite). A gas dispersion tube with fritted disc or cylinder is introduced through one neck. Attach electric heating mantle and water cooled condenser to other neck. Introduce anhydrous ammonia gas through the gas dispersion tube at a very low rate. Reflux the mixture for 6–8 hours. Filter, distill off excess benzene exercising care to prevent thermal decomposition of the guanidine. Purify by recrystallization from dry benzene or absolute ethanol.

#### EXAMPLE 5

(IV) The conversion of N,N' bis (4-dimethylaminophenyl) guanidine to N,N' bis (4-dimethylaminophenyl) carbodiimide via nitrous acid

Since the carbodiimides are highly reactive reagents and cannot be stored for prolonged periods this reaction is a simple expedient to facilitate the availability of reagents. The disubstituted guanidine can be converted to the corresponding carbodiimide by simply treating the guanidine with nitrous acid at low temperatures.

The removal of ammonia from guanidine, which accomplishes the same result (the formation of the carbodiimide), occurs with 80–90% yield with nitrous acid. See Smith, P.A.S., The Chemistry of Open Chain Organic Nitrogen Compounds, W. A. Benjamin Inc., New York, 1965, p. 258.

Since the dyes used herein serve two purposes: both as the sensitizer/sensitive media and as the coupler/developer color former there are two major restrictions on their structures:

(1) Sensitizer/sensitive media.—In this sense the dyes must conform to the structural limitations of the cyanine series sensitizing dyes. These limitations can be generalized as follows:



In which the pentavalent nitrogen is normally contained in a ring structure and the trivalent nitrogen can either be linear (open chain) or contained in a ring structure. In all cases there is an odd number of carbon atoms between the trivalent and pentavalent nitrogen atoms, with

alternating single and double bonds (resonant structures). The structures can be weighted to shift the spectral absorption by the addition of vinyl groups between the nitrogen atoms i.e.  $-\text{CH}=\text{CH}-$ . It should also be understood that  $-\text{C}\equiv$  is equivalent to and interchangeable with  $-\text{N}=$  therefore some of the atoms in the chain can be nitrogen. The nitrogen containing structures can contain in addition, atoms of oxygen, sulfur, or selenium provided they are not interposed in the direct chain between the two nitrogen atoms.

Alternately the compounds can also be of the merocyanine family with the following structural restrictions: Merocyanines



20

In which the trivalent nitrogen and keto groups can be in linear (open chain) or contained in ring structures. In all cases there is an even number of carbon atoms between the trivalent nitrogen and the keto group, with alternating single and double bonds (resonant structures). These structures can be weighted to shift the spectral absorption by the addition of  $(-\text{CH}-\text{CH})_n\equiv$  groups between the nitrogen and keto structures. It should also be understood that  $-\text{C}\equiv$  is equivalent to and interchangeable with  $-\text{N}=$  therefore some of the atoms in the chain can contain in addition, atoms of oxygen, sulfur, or selenium, provided they are not interposed in the direct chain between the nitrogen and keto groups.

25

30

35

These structures are resonant between the two extremes shown in the following:



50

55

(2) After exposure and fragmentation of the guanidine structure or portion of the structure the residual coupler structure must be suitable for coupling under alkaline conditions with the oxidized paraphenylene diamine (quinone diimine). The dyes formed in the light struck image areas to produce either the equivalent color (direct positive) or complementary color (negative) image.

#### Cyan couplers

The majority of cyan couplers currently in use are of the phenol class which yield indoaniline dyes. Including:

- 1-naphthol  
 1-thionaphthol  
 2,4-dichloro-1-naphthol  
 naphthols with 2,4,5,6-substituents  
 3,5-dibromo-o-cresol  
 4-chlorophenylphenol  
 m-hydroxybiphenyl  
 5,7-dibromo-8-hydroxyquinoline  
 Dihydroxydiphenyl methanes  
 1-hydroxy-2-naphthoyl-o-chloranilide  
 p-Niteobenzylpyridinium chloride  
 3-hydroxyguanazopyrazolone  
 Naphthaquinoline (with B substituted auxochrome)  
 Hydroquinone monomethylether



The commonly used condensing agents include: trialkylamines, trimethylamine, triethylamine, tri-N-propyl amine, tri-N-butyl amine, diethylmethylamine, ethyldimethylamine, quinoline, pyridine, isoquinoline, dialkylamines, sodium carbonate, and potassium carbonate.

In the case where one is reacting the highly reactive carbodiimides with an amino group in the intermediate the following generalization holds: Reactions in which carbodiimides are used are usually carried out under mild conditions at room temperature, or at a slightly higher temperature, with the use of such accessible solvents as ether, pyridine, or dimethyl formamide. The reactions, as a rule, do not take more than a few hours.

In terms of economics the Guanidine synthesis is much cheaper as the N,N' bis (p-dimethylaminophenyl) carbodiimide has a high commercial price. The storage problems associated with carbodiimides are serious since they are highly reactive, tend to polymerize, and therefore have very short shelf lives. As an intermediate in the synthesis of equivalent guanidines, which have long shelf lives, they are convenient.

A synthetic procedure will now be set forth illustrating the guanidine synthesis. The resulting dye is a double merocyanine with both keto groups contained within a single ring structure. The two groups are isolated in a bonding sense.

#### EXAMPLE 6

##### (V) Guanidine synthesis of a merocyanine dye

Condensation product of N,N' bis (4 - dimethylamino-phenyl) guanidine and 2,5-dichloro-p-benzoquinone<sup>1</sup>

Equations:



In a 500 ml. balloon flask, mix 100 ml. (78.9 g.) absolute ethanol, 59.4 g. N,N' bis (4-dimethylaminophenyl) guanidine (from preparation IIIa or IIIb), 17.7 g. 2,5-dichloro-p-benzoquinone (EK 4410), 6 g. magnesium oxide (BA 2477). Attach water cooled condenser, electric heating mantle, magnetic stirring unit, and reflux the mixture for 2 hours. Filter to remove solids, distill off ethyl alcohol, wash residue with distilled water, and dry. Purify by recrystallization from dry ethanol.

The resultant dye is magenta color in methanol solutions. After forming the silver salts, exposure, fuming of the guanidine portions of the structure, and coupling the resultant dye is cyan color in methanol solution.

The formation of silver or silver halide salts of these dyes follow the conventional methods currently in use in the manufacture of silver halide film. These processes involve the introduction of silver nitrate into the mixture and subsequent introduction of soluble halide salts (KI, KBr, KCl, NaI, NaBr, NaCl) followed by washing with water.

#### EXAMPLE 7

The following reaction will demonstrate the technique and simplicity in the formation of cyanine dyes using carbodiimides as reactants.

5 The intermediate, 2-amino-quinoline, is obtained from: Gallard-Schlesinger Chemical Mfg. Corp., Carle Place, L.I., N.Y. or K&K Laboratories.

The intermediate is then converted to a cyclammonium quaternary base in accordance with the procedures shown at par. 285 of Glafkides. The procedures are general and in this case we use CH<sub>3</sub>I as the alkyl halide. With this reaction completed we proceed as follows:

##### (VI) Carbodiimide synthesis of a cyanine dye

Condensation product of N,N'bis (4-dimethylamino-phenyl) carbodiimide<sup>1</sup> and 2-aminoquinoline methyl iodide.<sup>1</sup>

Equations:



In a 100 ml. balloon flask equipped with a stopper, mix 5 g. of dry calcium chloride (BA 1308), 25 ml. (17.7 g.) of anhydrous ether (BA 9244), 1.0 g. N,N'bis (4-dimethylaminophenyl) carbodiimide (K&K Labs #12325), and 1.0 g. of 2-aminoquinoline methyl iodide (K&K Labs #15039). The mixture is stirred while remaining at room temperature for approximately 2 hours. Filter to remove drying agent, distill off ether, and dry. Purify by recrystallization from ethanol.

The initial color of this dye is approximately magenta. After exposure and appropriate processing the resultant image is magenta.

Of the vast number of structures of the foregoing type which may thus be used in the invention, it will be evident that only three are required to produce subtractive or additive colors in an imaging member. Thus, for example, a reversal positive monopack (integral tripack) color film is structured as shown in FIG. 1. The schematic cross-section of the member 1 therein is broken at the middle to depict a first portion (a) illustrating the condition of member 1 prior to processing, and a second portion (b) illustrating the condition of member 1 subsequent to processing. From the direction of light exposure (top of figure) the member 1 at portion (a) is thus seen to consist of a blue light-sensitive layer 2a, yellow filter layer 4a, a green/blue light-sensitive layer 6a, a red/blue light-sensitive layer 8a, a transparent support 10a, and a dyed anti-halation layer 12a. After processing at (b), the corresponding structure consists of a blue absorbing layer 2b, a clear layer 4b, a green absorbing layer 6b, a red absorbing layer 8b, the support 10, and a clear layer 12b. It should be obvious that with judicious selection of the dye coupler portion Z of the cyanine sensitizer that either direct or complementary colors can be produced utilizing the same development process. The utilization of a single organic salt cyanine sensitizer as the sensitive salt, sensitizer, dye former-coupler and dye former-developer, with

13

in situ formation of the dye image associated with the wavelength portion of the original light image to which a selected coordinate structure is sensitive, now makes possible a color imaging structure employing but a single sensitive layer. Such a vastly simplified structure 14 is schematically depicted in the cross-sectional view of FIG. 2, and is seen to include a transparent support 15 upon which is coated a sensitive layer 17. The layer 17 includes a clear binder—which may constitute a clear plastic such as polyvinyl alcohol or other permeable resins, in which is dispersed in common a plurality of classes of organic structures of the type set forth herein. Thus in the simplest case three such classes of coordinate structures are commonly present in layer 17, each of said classes being respectively sensitive to a primary color component of a light image made incident upon member 14. In such simplest case the dye that results after processing each specific class of coordinate structures—i.e. after the coupler Z in each class structure couples with its developer-color former fragments  $\Delta$ NH—may have color reflective characteristics substantially identical with that color component of the original image to which the said coordinate structure is sensitive. In other cases the resulting dye, however, may be partially or entirely absorptive of wavelengths corresponding to the actinic wavelengths, selection of appropriate coordinate structures to yield desired dyes being a matter of choice dictated by the color balance characteristics desired in a given system.

In accordance with the present invention, development of exposed members such as those of FIGS. 1 and 2 is brought about by the extremely simple technique of heating the members Z (typically to from about 100 to 200° C.) or treating the sensitive layers with strongly alkaline buffered aqueous solutions (pH of the order of 10 to 13). Such environmental conditions will in the manner that has been previously set forth, serve to fracture the C—NH bonds in the dye coordinate structures, thus permitting coupling of the Z dye intermediates with fragments  $\Delta$ NH at those points in the sensitized layer where actinic radiation has activated the cyanine dye structures. Where heat is thus utilized as the energizing source for bond fracturing, any convenient method may be employed for applying such heat—including irradiation of the imaging member with infra-red energy from a lamp or similar source, or heating may be accomplished through use of microwaves or the like. Following the development step, the sensitized layers of the imaging member will typically be washed in a solution of water and acetic acid (stop), bleached to remove metallic silver, fixed with conventional hypo solution, washed to remove silver complex, and thereupon the member is dried.

While the present invention has been particularly set forth in terms of specific embodiments thereof, it will be appreciated in view of the instant disclosure, that numerous variations upon the present invention are now enabled to those skilled in the art, which variations are yet in proprietary within the scope of the instant teaching. Accordingly the invention is to be broadly construed, and limited only by the scope and spirit of the claims now appended hereto.

1. A method for photographic color imaging, comprising:

(a) exposing to an image pattern a sensitized layer containing cyanine dye coordinate structures of the type



14

where M is a silver ion, and n is an integer, said structure being chosen to be light sensitive to a selected color component of said light pattern, where Z is a dye coupler for the developer-color former fragment  $\Delta$ NH and which when coupled with said fragment yields a dye having a desired color relationship to said selected color component of said incident image pattern, impingement of light including said selected color component serving to reduce said silver ion and oxidize said developer fragment;

(b) disrupting the chemical bonds joining said developer fragments to said structure, whereby said dye coupler couples with said oxidized developer fragments at points exposed to said selected color component; and

(c) removing reduced metal and metal complexes from said emulsion.

2. A method in accordance with claim 1, wherein  $\Delta$ NH is a double substituted paraphenylene diamine.

3. A method in accordance with claim 2, wherein said dye resulting from said coupling action is substantially identical in color to said selected color component.

4. A method in accordance with claim 2, wherein said dye resulting from said coupling action is substantially optically absorptive of said selected color component.

5. A method in accordance with claim 2, wherein said chemical bonds are disrupted by heating said layer containing said coordinate structures.

6. A method in accordance with claim 2, wherein said chemical bonds are disrupted by treating said layer containing said coordinate structures with an alkaline solution.

7. A member for photographic color recording of a light image pattern exposed thereto, comprising:

(a) a support substrate; and

(b) a binder layer containing cyanine dye coordinate structures of the type



where M is a silver ion, and n is an integer, said structure being chosen to be light sensitive to a selected color component of said light pattern, when Z is a dye coupler for the developer fragment  $\Delta$ NH and which when coupled with said fragment yields a dye having a desired color relationship to said selected color component of said incident image pattern, impingement of light including said selected color component serving to reduce said silver ion and oxidize said developer fragment whereby disruption of the chemical bonds joining said developer fragments to said structure enables coupling of said oxidized fragments to said dye coupler at points exposed to said selected color component.

8. A member in accordance with claim 7, wherein  $\Delta$ NH is a double substituted paraphenylene diamine.

9. A member in accordance with claim 8, wherein said dye resulting from said coupling action is substantially identical in color to said selected color component.

10. A member in accordance with claim 8, wherein said dye resulting from said coupling action is substantially optically absorptive of said selected color component.

11. A member in accordance with claim 8, including a plurality of species of coordinate structures of said type, each said species included in said plurality being associated with a specifically selected of said color components.

12. A member in accordance with claim 11, wherein three said species are present, each said species being associated with a primary color of the visible spectrum.

13. A member in accordance with claim 11, wherein each of said species is present in a distinct layer of said member.

14. A member in accordance with claim 11, wherein said plurality of species are commonly present at points in a single layer.

## References Cited

## UNITED STATES PATENTS

3,453,107 7/1969 Idelson ----- 96-29 D

5 RONALD H. SMITH, Primary Examiner

U.S. Cl. X.R.

96-66 R, 74, 114.1, 114.6